

March 22, 1960

C. H. SCHUH

2,929,756

PRODUCTION OF BAMBOO PULP AND PAPER

Filed Jan. 23, 1958



*inventor*  
Charles Herman Schuh

By *Hill, Sherman, Meroni, Gross & Simpson Atty's.*

# United States Patent Office

2,929,756

Patented Mar. 22, 1960

1

2,929,756

## PRODUCTION OF BAMBOO PULP AND PAPER

Charles Herman Schuh, Tampa, Fla., assignor to  
the Government of Burma

Application January 23, 1958, Serial No. 710,809

6 Claims. (Cl. 162—26)

This invention relates to an improved method and apparatus for the production of bamboo pulp and paper products, and more particularly, to an improved method and apparatus for modified mechanical pulping of bamboo.

It has been stated in the literature and by various research investigators that mechanical pulping of bamboo is not practical or feasible. For example, after an extensive investigation by the Herty Foundation, it was reported that "Most of the known methods of pulping have been applied to bamboo. Least promising of the conventional methods is mechanical pulping."

U.S. Patent No. 1,376,789 describes a machine for shredding bamboo based on a combined cutting and splitting action for producing slivers of bamboo for use in brooms or the like. A machine has also been proposed for shredding bamboo for paper and pulp production which involves shredding of pieces of bamboo by rubbing apart and cutting across the fibers with saw teeth and the like. There is a general reduction of the pieces to a comminuted mass. These and other devices have been proposed but each has left much to be desired for practical use with bamboo.

The present invention avoids the problems and drawbacks of conventional mechanical pulping, as applied to bamboo. The instant invention makes it possible not only to successfully and economically produce mechanical bamboo pulp but also to produce a pulp that is superior to mechanical wood pulp. In addition, the instant invention produces a mechanical bamboo pulp at lower cost than that required for producing mechanical wood pulp. The superiority of the instant bamboo pulp results from a much greater average fiber length, a higher ratio of fiber length to fiber diameter and improved ease of hydration of the fiber.

In the practice of the instant invention it is possible to individualize the fibers by a bearing and combing out of the pith between the fibers. The instant invention differs from the usual or conventional carding process which employs relatively thin teeth spaced closely together for literally combing out the fiber. In contrast, in order to achieve the desired result of the instant invention, it is necessary to provide a rotating drum of certain size, with teeth of a definite size and shape, spaced in a particular manner and with a definite speed of rotation, using a definite speed and manner of feeding the bamboo culms against the rotating drum. The action against the culms resulting in the practice of the instant invention is a combination of impact, attrition, and combing.

It is, therefore, an important object of the instant invention to provide an improved method and apparatus for producing bamboo pulp and paper.

Another important object of the instant invention is to provide an improved apparatus for producing bamboo pulp comprising a rotary drum, means for rotating said drum, a myriad of short dull closely spaced teeth projecting radially from the drum surface, and means for feeding bamboo culms against the teeth on the rotating drum surface generally tangentially to the drum surface.

2

Still another important object of the instant invention is to provide an improved process of producing bamboo pulp comprising the step of subjecting bamboo culms having a moisture content in excess of 40% to a shredding action produced by 8,000 to 12,000 longitudinal tooth strokes per inch width per inch feed of bamboo to individualize the fiber and cut it into lengths averaging largely between  $\frac{3}{8}$  inch and 1 inch.

Other and further features, objects and advantages of the present invention will become apparent to those skilled in the art from the following detailed disclosure thereof and the drawing attached hereto and made a part hereof.

On the drawings:

Figure 1 is an essentially diagrammatic elevational view showing the device of the instant invention;

Figure 2 is a detail view of an individual tooth in the device of the instant invention; and

Figure 3 is a view in perspective of the drum employed in the instant device, with certain associated parts.

As shown on the drawings:

The device of the invention, indicated generally at 10 in Figure 1, comprises a rotary drum 11, a motor indicated diagrammatically at 11b for rotating the drum 11, a myriad of short dull closely spaced teeth 12 projecting radially from the drum surface, and means (indicated at 13) for feeding bamboo culms B against the teeth 12 on the rotating drum surface generally tangentially to the drum surface. Such means 13 being indicated here has a motor 13a driving a worm gear 13b which moves a screw 13c axially and the screw 13c mounts a backing member 13d at one end thereof for urging the bamboo culm B against the teeth 12 at a predetermined rate.

As indicated in Figure 2, each tooth 12 has an average radial dimension R of  $\frac{1}{2}$  inch to 1 inch, the radial dimension here shown being  $\frac{3}{4}$  of an inch. Each tooth 12 has an average dimension d at its base of  $\frac{1}{16}$  inch to  $\frac{1}{4}$  inch; and the tooth 12 here shown has a diameter of  $\frac{3}{16}$  inch. The tooth 12 is tapered at its outer extremity 12c to give relatively dull knife edges 12b.

Referring to Figure 3, it will be seen that the drum 11 has a relatively large diameter of 2 to 3 feet and there is a relatively high density of teeth 12 on the peripheral surface 11a of the drum 11. The teeth 12 are shown in full view near the top of the drum 11 in Figure 3, but for the sake of simplicity the remaining teeth on the surface 11a are omitted in Figure 3 and dots 12a are shown indicating the location of the centers of each of such other teeth. The dots 12a bring out more clearly the nature of the density of the teeth, which is herein defined as the number of teeth in a given area on the peripheral drum surface 11a. For example, the dotted lines 14a and 14b on the peripheral drum surface 11a represent circumferences which are spaced apart 1 inch (longitudinally of the drum 11) and thus define a peripheral area A 1 inch in width on the drum surface. This peripheral area has an average tooth density of 128 to 256. In other words, the total number of teeth 12 whose centers lie within the peripheral area A may range from 128 to 256. The teeth 12 have a generally random arrangement, except for the fact that certain tooth densities have been found to be important. The actual tooth density for the peripheral area A in the instant drum is 192 teeth. Expressed in other terms, if circumferences (such as the circumferences 14a and 14b) are drawn on the drum surface  $\frac{3}{32}$  inch apart, there will be three teeth centered on each such circumference, when a 3 foot diameter drum is used, such as the instant 3 foot diameter drum. Actually, an average of from 1 to 4 teeth may be centered on each such circumference, but this will require less advantageous rotating speeds for the drum and an average of 3 teeth is preferred.

The drum 11 is preferably driven so as to produce a

surface speed of 2,000 to 2,500 feet per minute. The best results are obtained using a surface speed of 2,200 feet per minute which is 250 revolutions per minute with a 3 foot drum. Such are the operating conditions here used.

The bamboo culm B is fed against the teeth 12 on the drum 11 generally tangentially to the drum 11 at a predetermined rate of about 4 inches to about 6 inches per minute. A certain number of tooth strokes for a given area of bamboo are required. Rotating the 3 foot diameter drum 11 at 250 r.p.m., it will be appreciated that in the peripheral area A, which is 1 inch in width, there are 48,000 tooth strokes per minute. These tooth strokes are, in effect, longitudinal of the bamboo culm. If the culm is fed at a rate of 6 inches per minute then each inch of bamboo fed receives 8,000 longitudinal tooth strokes per inch of width of the bamboo culm. It has been found that the best results are obtained using 8,000 to 12,000 longitudinal tooth strokes per inch width per inch feed of bamboo. The 12,000 longitudinal tooth strokes per inch width per inch feed of bamboo are obtained feeding at a rate of only 4 inches per minute.

It should also be noted that in a small peripheral area  $a$  of only 1 square inch, the average tooth density is 2. Two tooth centers 12a, 12a are shown in the inch square peripheral area  $a$  of Figure 3. The tooth density per square inch may vary from 1 to 3 teeth, but 2 teeth is the preferred tooth density, and this is the tooth density on the drum 11 here shown. Of particular importance, is the actual drum surface speed of 220 feet per minute. As the drum diameter is varied the tooth densities are varied to effect the desired number of tooth strokes at the drum surface speed of about 220 feet per minute.

It has been found that the instant shredding arrangement is carried preferably with bamboo culms having a moisture content of above 40 (weight) percent, and the best results are obtained using culms with a moisture content of at least 50%. Bamboo culms having a moisture content of less than 40% are first soaked in water to obtain the desired moisture content.

Under the instant shredding conditions superior results are obtained in the form of highly individualized fiber masses containing a minimum of powdered material and having an optimum average fiber length with very remarkably low power consumption. The percentage of powdered material (largely pith) is well below 10%. The average fiber length will be in the range of  $\frac{3}{8}$  inch to 1 inch, with relatively small amounts above 2 inches and below  $\frac{1}{4}$  inch. The power consumption is in the order of 10 to 20 horsepower per ton of bamboo per day (dry basis). This is only a small fraction of the power consumed in the conventional mechanical pulping of wood, which is about 60 to 100 horsepower per ton of wood ground per day.

It has further been found that the products of the instant shredding process can readily be converted to paper pulp stock by beating in the conventional type beater with certain precautions. The loading of the drum should be relatively light as the fibers cut easily. If the pH is held above 12 during beating it has been found that a sheet of greatly increased strength is obtained. For example, after 60 minutes of beating at a conventional pH of about 7, the breaking length of a test sheet was found to be 1.37 kilometers, whereas the same heating operation at a pH of 12.5 gives a test sheet having a breaking length of 2.70 kilometers, which is a gain of over 100% in strength. Also, the burst factor of sheets made from pulp using the conventional pH of 7 during beating was 0.20, whereas the burst factor for sheets made from pulp wherein the pH of 12.5 was maintained during beating is 0.44. This also represents a 100% gain in strength. It will be appreciated that these test sheets were made without any additions.

Since the instant shredder product cuts relatively easily the beating or pulping is carried out in a tank with high speed mixing. Fiber is reduced in length and further individualized and hydrated, as in the beater. In this instance, the pH may be conveniently maintained even higher than 12.5 with no harmful effects to the equipment, for example, by the addition of caustic up to 2%. The caustic soda thus used may range from  $\frac{1}{2}$  to 2%.

For a crude type of pulp, useful in hard board production, the shredded product is simply pulped in the beater for about 30 to 40 minutes to condition it, and then formed into sheets and hot pressed in the usual manner. A similar processing will be found suitable for some types of cardboard and the like. In this instance, the time of pulping may be extended somewhat and the pH raised to above 12. Other additions may be made in line with the usual practice for this type of product. In the case of finer grades of pulp and paper stock, it is advantageous to first screen the shredded product to remove the powdered portion which is largely pith and non-fibrous node particles. The non-fibrous powdered portion is less than 10% and it may be regarded merely as filler, if it is left in the shredded product.

If a particularly fine grade of pulp is desired, it is advantageous to raise the caustic content during pulping and to carry out this step at elevated temperatures with direct steam heating. It is not necessary to use pressure cooking with all its expensive problems and drawbacks. Open steel tanks with open coil direct steam heating and high speed agitators are sufficient. As previously indicated, comparatively low concentrations of caustic will suffice for most purposes (within the range of  $\frac{1}{2}$  to 2%). The chemical treatment, pulping, and conditioning for individualization of the fiber and partial hydration and reduction of fiber length are all accomplished at the same time with the simplest kind of equipment at a minimum of power consumption. Excess unused caustic is recovered by washing the fiber in the usual manner.

The washed fiber may be screened in the usual manner to obtain high quality pulp, which may also be subjected to a bleaching action using, for example, zinc hydrosulphite, as in the case of mechanical wood pulp. The instant pulp stock may be given a final beater treatment to more completely hydrolyze the fiber and to make the usual sizing and loading additions for specific types of paper. Sheet formation is carried out in the conventional manner for wood pulp.

The shredded product of the instant invention is unique in that it may be used in conventional wood pulp beating, conditioning, and the like operations including sheet formation. The instant pulp is advantageously suggested to pulping and beating at a pH of 12 or more.

It will be understood that modifications and variations may be effected without departing from the spirit and scope of the novel concepts of the present invention.

I claim as my invention:

1. The process of producing bamboo pulp and paper products comprising subjecting bamboo culms having a moisture content in excess of 40% to a shredding action produced by 8,000 to 12,000 longitudinal tooth strokes per inch width per inch feed of bamboo to individualize the fiber and cut it into lengths averaging largely between  $\frac{3}{8}$  inch and 1 inch, said teeth having an average height of  $\frac{1}{2}$  to 1 inch and an average diameter of  $\frac{1}{8}$  to  $\frac{1}{4}$  inch, and producing less than 10% of powdered material of -100 mesh; then subjecting the shredded product to a mechanical pulping action in a water suspension of pH in excess of 12, followed by sheet formation from the pulp suspension by dewatering and felt-ing and pressing and drying to form finished sheets.

2. The process as claimed in claim 1, in which the shredded product is screened before pulping, in order to remove the powdered non-fibrous material.

3. The process as claimed in claim 1, in which the

pulping step is carried out using a suspension containing  $\frac{1}{2}$  % to 2% caustic soda.

4. The process as claimed in claim 1 in which the shredded product is screened to remove powdered non-fibrous material before pulping and in which the pulping 5 step is carried out in a suspension containing up to 2% of caustic soda, and in which the pulped fiber is washed and screened to remove excess caustic and any undesirable particles still remaining prior to sheet formation.

5. The process as claimed in claim 4, in which the 10 washed and screened pulp is given a bleaching treatment with zinc hydrosulphite prior to sheet formation.

6. The process as claimed in claim 5, in which the washed, screened and bleached pulp is given a second beater treatment to more completely hydrolyze the fiber 15 and this is followed by making various sizing and loading additions prior to sheet formation.

References Cited in the file of this patent

UNITED STATES PATENTS

|           |           |       |               |
|-----------|-----------|-------|---------------|
| 254,958   | Guest     | ----- | Mar. 14, 1882 |
| 635,436   | Fritz     | ----- | Oct. 24, 1899 |
| 1,344,180 | McMillan  | ----- | June 22, 1920 |
| 1,549,103 | Barnes    | ----- | Aug. 11, 1925 |
| 1,726,078 | Leyst     | ----- | Aug. 27, 1929 |
| 1,813,184 | McQuiston | ----- | July 7, 1931  |
| 1,847,050 | Williams  | ----- | Feb. 23, 1932 |

FOREIGN PATENTS

|         |               |       |               |
|---------|---------------|-------|---------------|
| 503,960 | Italy         | ----- | Dec. 9, 1954  |
| 733,364 | Great Britain | ----- | July 13, 1955 |